

Nov. 29, 1960

A. W. SCRIBNER

2,962,164

METAL EXTRUSION

Filed Dec. 14, 1959

2 Sheets-Sheet 1



Fig. 3



Fig. 2



Fig. 1

Albert W. Scribner

Nov. 29, 1960

A. W. SCRIBNER

2,962,164

METAL EXTRUSION

Filed Dec. 14, 1959

2 Sheets-Sheet 2



Fig. 4



Fig. 5



Fig. 6



Fig. 7



Fig. 8

Albert W. Scribner

2,962,164

## METAL EXTRUSION

Albert W. Scribner, 89 Grennan Road,  
West Hartford 7, Conn.

Filed Dec. 14, 1959, Ser. No. 859,325

7 Claims. (Cl. 207—10)

This invention relates to an improved method of die expressing metal and more particularly relates to a novel method for timing and locating the extrusion forces applied to a work billet.

This application is a continuation-in-part of my co-pending applications Serial Nos. 630,962 and 630,963, both filed on December 27, 1956, and both entitled "Metal Extrusion," and both now abandoned.

In conventional types of metal extrusion operations, such as that generally illustrated by U.S. Patent 2,335,590, some of the work material, namely that initially located radially outward from the limits of the die opening, must convergently flow toward the die opening before it can be extruded through said opening. Simultaneously the metal initially located nearer the billet axis flows in a direction which is more nearly parallel to the die axis before it passes through the die orifice. It will be noted that as the working ram advances that portion of the billet nearest the die axis flows through the die orifice more readily than that portion of the billet located radially more remote from said axis. This prominent axial flow sharply curbs or restrains the convergent metal flow thereby causing the billet to be greatly distorted before it can be fully extruded. This distortion is accompanied by a large amount of internal turbulent flow in the work metal which in turn requires the application of excessively high working forces to effect the extrusion operation.

One object of the instant invention is to provide a novel method for die expressing a work billet whereby the amount of turbulent metal flow may be substantially reduced.

Another object of the invention is to provide a method for sequentially controlling the convergent and axial flow of the billet material during the extrusion operation.

Another object of the invention is to provide a method for sequentially die expressing a metal billet in two or more extrusion strokes whereby the total effective working stroke for the overall extrusion operation may be increased to a length greater than the initial length of the work billet.

Another object of the invention is to provide a novel method for serially die expressing different longitudinal portions of the work billet using two or more consecutive extrusion strokes whereby the interference between the convergent and axial flow of the billet material is greatly reduced.

Another object of the invention is to provide a novel method for more efficiently extruding a metal billet whereby the convergent metal flow is produced by a forging action and the axial metal flow is produced by an extrusion action.

A further object of the invention is to provide a metal extrusion method wherein the energy required to die express a given size billet is much less than that required when using conventional methods.

Other objects and many of the attendant advantages of

this invention will be readily appreciated as the same becomes better understood by reference to the following detailed description when considered in connection with the accompanying drawings in which like reference numerals designate like parts throughout the figures thereof and wherein:

Figures 1, 2 and 3 are axial sectional views showing the sequential operation of the principal parts of a metal extrusion press which can be used to carry out the instant method.

Figures 4, 5, 6, 7 and 8 are axial sectional views of the principal parts of a metal extrusion press which can be used to carry out two variations of the instant method.

Referring to Figure 1 there is shown a conventionally supported container 1 which is adapted to receive and position a work billet. A tubular ram 2 is slidably mounted at the lower end 7 of said container. On the inner end of ram 2 there is operatively secured an extrusion die 5 having an orifice 6 formed therethrough. The cross sectional profile of ram 2 is preferably circular and has an effective area which is considerably less than that of the billet receiving chamber in the container 1. At the other end 8 of the container there is slidably mounted a ram 9 which has a work engaging face 10 and a tubular shank portion 11. The ram 9 is substantially coaxially disposed with respect to both the container 1 and the ram 2. Rams 2 and 9 may be power driven by any suitable means such as hydraulic motors having controls for effecting the respective sequential actuation of the rams as hereinafter described.

In operation the rams 2 and 9 are withdrawn and a work billet is inserted in the work receiving chamber of container 1. The rams are then advanced to their initial operative positions shown in Figure 1 wherein the respective operative faces of the rams engage the ends of said work billet. Thereafter ram 9 is held fixed relative to container 1 while ram 2 is advanced through a working stroke  $E_1$ , as shown in Figure 2, to centrally pierce the end of the work billet and thereby indirectly die express the central longitudinal portion of the billet. The cross sectional area of this central longitudinal billet portion is greater than the cross sectional area of the die orifice 6. As the volume of the central portion of the billet is thus being reduced the volume of the substantially unworked outer longitudinal portion of the billet remains substantially constant. Subsequently, while container 1 remains stationary, ram 2 is withdrawn through a stroke  $E_2$  and ram 9 is simultaneously advanced through a working stroke  $E_3$  as shown in Figure 3 to thereby die express the remaining tubular portion of the work billet. The relative speeds of the rams 2 and 9 during their respective working strokes  $E_2$  and  $E_3$  are such that the volumetric displacement rate of ram 9 always exceeds that of ram 2; i.e. the volume of the work billet is continually being reduced during said strokes  $E_2$  and  $E_3$  thereby insuring a continuous die expressing of the work material. The stroke  $E_3$  is preferably started just prior to the termination of stroke  $E_1$  so that there is no interruption of metal flow through the die orifice 6 during the transition between the extrusion stages. Further, the amounts of the respective volumetric displacements of the rams 2 and 9 may be controlled so that the actual extrusion of the work metal continues at a substantially constant rate.

The cross sectional size of ram 2 may be adjusted so that the maximum and average forces required to execute the first stage extrusion stroke  $E_1$  most nearly correspond to the maximum and average forces required to execute the second stage extrusion strokes  $E_2$  and  $E_3$ . In this way the greatest operative force requirements occurring at any time are reduced to a minimum value. The ex-

trusion strokes  $E_1$  and  $E_2$ ,  $E_3$  may each be shortened whereby a plurality of alternate shortened strokes corresponding to strokes  $E_1$  and  $E_2$ ,  $E_3$  may be used to successively extrude several shorter radially inner and outer longitudinal portions of the billet to thereby complete the die expressing of the billet.

By applying extrusion forces to the billet in two distinct extrusion stages as described above several advantages are obtained. First, the sequential displacement through die aperture 6 of the billet portions respectively located relatively near and relatively remote from the axis of said die aperture reduces the amount of billet distortion normally associated with conventional types of extrusion operations. This will reduce the amount of internal turbulence in the work material and such will decrease the amount of energy required to extrude the billet. Secondly, it will be noted that the total effective length of the two consecutive extrusion strokes  $E_1$  and  $E_2$ ,  $E_3$  is much greater than the initial length of the billet. By using such a longer effective operative stroke the extrusion of the billet will be efficiently "geared down" so that the amount of mechanical energy required to extrude the billet may be delivered by the application of much smaller forces and as a result the structural elements of the press will be subjected to much smaller working stresses whereby the overall construction of the press may be substantially lightened. Thus the initial, operating and maintenance costs for an extrusion press having a given required capacity may be greatly reduced.

It will be noted that there is no sliding friction between the billet metal and the inner longitudinal walls of the container 1; the only relative movement between the billet metal and the longitudinal surfaces of the tools occurring over the relatively small outer surfaces of ram 2. Also any scale or imperfections in the outer skin of the billet are not extruded during the stroke  $E_1$ . It will be apparent that the work billet will assume the cylindrical shape of the work receiving chamber of the container 1 and will thus have a substantially uniform outer cross sectional profile during the working operations. With reference to the apparatus shown, the extrusion die 5 may be mounted on ram 9 instead of on the ram 2, and the relative movement between the rams 2 and 9 and/or the container 1 may be respectively effected by the proper axial displacement of said container relative to one or both of said rams. Also a conventionally supported and actuated mandrel may be used with either of the two disclosed types of presses when it is desired to produce tubular extrusions from a tubular or pierced work billet.

Two modifications of the instant method are respectively illustrated in Figures 4-6, and Figures 7 and 8. Referring to Figures 4-6 there is shown a conventionally supported container 15 having a cylindrical bore or chamber 16 which is adapted to receive and support a work billet. Slidably mounted at the open end of container 15 are two coaxial and telescopically disposed tubular working rams 17 and 18. At the inner end of ram 18 there is operatively secured an extrusion die 19 having an orifice 20 formed therethrough. The rams 17 and 18 may be respectively power operated by hydraulic motors having suitable controls for effecting the herein-after described sequential operation.

In the extrusion operation illustrated in Figures 4-6 the rams 17 and 18 are withdrawn and a work billet is inserted in the chamber 16 of the container. The rams are then advanced to their respective initial positions shown in Figure 4 wherein the inner ram faces engage the end of the billet. The ram 17 is then held substantially fixed relative to the work billet while the ram 18 is advanced through a short extrusion stroke  $P$  as shown in Figure 5 to thereby pierce and reduce the volume of the central portion of billet. As will be apparent the cross sectional area of this central billet portion will be greater

than that of the extrusion die orifice 20. During the extrusion stroke  $P$  the volume and shape of the substantially unworked tubular peripheral portion of the billet material will remain substantially the same. The ram 17 is then advanced through a short forging stroke  $F_1$  while the ram 18 is simultaneously retracted through a short stroke  $F_2$  as shown in Figure 6 to thereby displace a part of the peripheral portion of said billet material towards the billet axis and nearer axial alignment with the die orifice. The rates and amounts of the respective volumetric displacements for the rams 17 and 18 during the said strokes  $F_1$  and  $F_2$  are substantially equal and hence the volume of said billet immediately before, during and immediately after the execution of strokes  $F_1$  and  $F_2$  is substantially the same. As a result there will be substantially no die expressing of the work metal during these working strokes; rather the unextruded metal will be forged or reshaped so as to cause a radial outer portion thereof to convergently flow towards the billet or die axis preparatory for a subsequent extrusion stroke. The extrusion stroke and the forging stroke are then alternately repeated until the die expressing of the billet is completed. The ram 17 preferably commences its forging stroke  $F_1$  just prior to the completion of the extrusion stroke  $P$  so that there is no hesitation or interruption in the application of the working forces; likewise the second extrusion stroke preferably commences just prior to the completion of the next preceding forging stroke. Here again the effective cross sectional areas of the rams 17 and 18 may be adjusted so that the maximum forces required to effect the extrusion operations are substantially the same as the maximum forces required to effect the forging operations. In this way the largest force required at any time during the working operations will be reduced to a minimum value.

By utilizing the method described in connection with Figures 4-6 the amount of turbulent internal metal flow, and hence the total amount of mechanical energy required to die express a given work billet, is reduced because a substantial part of the interference between the above noted convergent and axial metal flow patterns is eliminated. The convergent flow of the work metal, instead of tending to choke the extrusion action as in conventional extrusion operations, here takes place during a forging operation which is separate from any substantial axial metal flow and which requires the application of working forces that are much less than the high extrusion forces normally required to produce the simultaneous and mutually interfering convergent and axial flow of the radially outer and inner portions of the unextruded material. The reduced amount of mechanical energy necessary here to complete the extrusion operation is a product of force times distance and may be obtained by the application of still further reduced maximum forces in that again a relatively long working stroke is used, the combined length of the extrusion strokes such as  $P$  being much greater than the initial length of the billet. As before this permits a press of a desired capacity to have a far lighter construction and a much smaller power operating means. It will be noted in Figures 4-6 that the extrusion forces exerted by ram 18 during stroke  $P$  are applied in a manner to directly localize the high extrusion pressures in that region of the billet which is radially as well as axially adjacent the die orifice; thus the high unit extrusion pressures are not dispersed and dissipated through the whole billet before they act on that portion of the billet material which is about to be die expressed.

Instead of starting the working operations with an extrusion stroke  $P$  as shown in Figure 5, the rams 17 and 18 may be moved from their respective initial positions to those shown in Figure 7 to thereby initially effect a forging operation wherein a peripheral portion of the billet is displaced towards the billet axis to form a reduced axial extension. Here the ram 17 is advanced through a

short stroke  $F_3$  while ram 18 is simultaneously retracted through a stroke  $F_4$ . Again the rates of volumetric displacements of rams 17 and 18 are substantially the same so that there is substantially no metal flow through the die orifice 20 during this billet reshaping operation. Thereafter ram 17 is held fixed relative to the unextruded billet material while ram 18 is advanced through a short extrusion stroke D as shown in Figure 8 to thereby die express a central portion of the billet material. At the end of stroke D the inner face of ram 18 may be slightly above or below the inner face of ram 17. These forging and extruding steps are alternately repeated until the die expressing of the work metal is completed.

In Figures 4-8 a displacement of the working rams 17 and 18 relative to the container 15 is used to effectuate the billet working strokes, however it will be apparent that the container 15 may be properly moved relative to one or both of the same in order to effect one or more of the working strokes. In order to insure that no unfilled container space exists during the forging strokes  $F_1$  and  $F_2$  of Figure 6, for example, the rate and amount of volumetric displacement for the stroke  $F_1$  may be made slightly greater than that for stroke  $F_2$  whereby a very slight amount of extrusion of the billet will occur during the forging operations. The die 19 may be operatively mounted in the upper end wall of the container 1; and the rams 17 and 18 may be mounted at opposite ends of the container with the die operatively secured to either of said rams.

While several embodiments of the invention have been shown and described, it will be apparent to those skilled in the art that numerous variations and modifications may be made in the particular construction without departing from the underlying principles of the invention. It is therefore desired, by the following claims, to include within the scope of the invention all such variations and modifications whereby substantially the results of the invention may be obtained by the use of substantially the same or equivalent means.

The invention claimed is:

1. A method of die expressing a work billet of solid metal which has a substantially uniform cross section and which is operatively confined adjacent an extrusion die orifice; comprising the steps of die expressing a radially central portion of said billet through said orifice by longitudinally and centrally piercing one end of said billet, the cross sectional area of said central portion of said billet being greater than that of said orifice, and die expressing substantially the remaining radially outer tubular longitudinal portion of said billet by applying an extrusion force to the unextruded portion of said billet.

2. The method defined by claim 1 wherein the volume of the work material in said outer tubular billet portion remains substantially constant during the first mentioned die expressing step.

5 3. A method of die expressing a work billet of solid metal which has a substantially uniform cross section and which is operatively confined adjacent an extrusion die orifice; comprising the successive steps of centrally piercing said billet and indirectly die expressing substantially the central portion of said billet through said orifice by applying an extrusion force to just the center part of the billet end cross section, and die expressing substantially the remaining tubular portion of said billet by applying an extrusion force to the unextruded outer portion of said billet.

10 4. The method defined by claim 3 wherein the die expressing strokes are each shortened in length and are alternately repeated to successively extrude several shorter inner and outer portions of said work billet.

15 5. A method of die expressing a metal billet; comprising the steps of operatively confining the billet adjacent an extrusion die orifice, axially piercing one end of said billet to thereby die express a central portion of said billet, forging the unextruded billet material while keeping the volume thereof substantially constant so as to increase the amount of work material located near axial alignment with said die orifice, and axially piercing the reshaped unextruded material to thereby die express a central portion of the reshaped work material.

20 6. A method of die expressing a work billet; comprising the steps of operatively confining the billet adjacent an extrusion die orifice, reducing the volume of said work billet to thereby die express a portion of the work billet material through said orifice, reshaping the unextruded work material while keeping the volume thereof substantially constant so as to increase the amount of unextruded work material which is located near axial alignment with said extrusion die orifice, and reducing the volume of the reshaped work material to thereby extrude another portion of the work material through said die orifice.

25 7. The method defined by claim 6 wherein the reshaping step produces a reduced axial extension on the unextruded work material.

References Cited in the file of this patent

UNITED STATES PATENTS

|           |          |               |
|-----------|----------|---------------|
| 74,755    | Farrell  | Feb. 25, 1868 |
| 2,230,840 | Jongedyk | Feb. 4, 1941  |
| 2,920,760 | Genders  | Jan. 12, 1960 |